

Feb. 16, 1954

R. DOAT

2,669,446

CUPOLA FURNACE

Filed May 15, 1952

4 Sheets-Sheet 1



FIG. 1.

INVENTOR.

ROBERT DOAT  
BY

*Robert Doat*  
age

Feb. 16, 1954

R. DOAT

2,669,446

## CUPOLA FURNACE

Filed May 15, 1952

4 Sheets-Sheet 2



FIG. 3.

BY

INVENTOR.  
ROBERT DOAT

Michael Johnson  
age 1

Feb. 16, 1954

R. DOAT

**2,669,446**

## CUPOLA FURNACE

Filed May 15, 1952

4 Sheets-Sheet 3

FIG. 5.



INVENTOR.

ROBERT DOAT

BY

Michael S. Brown  
Sagittarius

FIG. 4.

Feb. 16, 1954

R. DOAT

2,669,446

CUPOLA FURNACE

Filed May 15, 1952

4 Sheets-Sheet 4

FIG. 7.



FIG. 8.

FIG. 6.



INVENTOR.

ROBERT DOAT  
BY

*Robert Doat*

## UNITED STATES PATENT OFFICE

2,669,446

## CUPOLA FURNACE

Robert Doat, Liege, Belgium

Application May 15, 1952, Serial No. 287,895

Claims priority, application Belgium July 17, 1951

12 Claims. (Cl. 266--30)

1

The present invention relates to cupola furnaces and processes for operating the same.

More particularly the present invention relates to a cupola furnace which is adapted to function also as a gas producer.

This application is a continuation-in-part of U.S. patent application Serial No. 165,420, filed June 1, 1950, and entitled "Process For Melting Metal Ores and Cupola Furnace Therefor", now abandoned.

In conventional cupola furnaces it is a fairly difficult matter to produce a uniform product of high quality. The reasons for this are, among others, that in attempting to conserve fuel there exists in the furnace an oxidizing atmosphere which results in oxidation of various elements in the charge so that an inferior product is produced. Moreover, because of this oxidation and because of mixing of the slag bath with the materials of the refractory lining, it is impossible to accurately control the slag through which the molten metal passes.

Because the operator is not the master of the molten slag within the furnace, he cannot control the product produced. The reason for this is that the molten metal passing through the slag bath reacts with the slag bath, and this reaction is uncontrollable when the slag itself cannot be accurately controlled.

Another disadvantage of conventional cupolas is that they cannot be operated continuously for long periods of time because the refractory lining deteriorates rapidly, and it thus becomes necessary to interrupt the operations and repair the lining. For example, with a conventional cupola which has an output of 20 tons of molten metal an hour, it is seldom possible to exceed 10 hours of continuous operation. After this time it is necessary to repair the refractory lining above and below the melting zone.

This conventional type of cupola, which may be used either in an iron or steel foundry, is generally provided with one or two ranges of rectangular tuyeres. The ratio between the horizontal cross-section of the interior of the cupola and the sum of the cross-sections of the tuyeres varies between 5 and 12. The air pressure at the tuyeres is generally low, being in the

2

neighborhood of 25 cm. of water above atmospheric pressure for a cupola producing 2 tons of metal per hour and in the neighborhood of 60 cm. of water above atmospheric pressure for a cupola producing about 10 tons of metal per hour. In such conventional cupolas the speed of air flowing through the tuyeres is generally about 20 meters per second. Under these conditions the gas which flows from the top of the cupola has a calorific content below 200 calories per cubic meter and the ratio of CO to CO<sub>2</sub> in this gas is from 0.4 to 0.6. The molten metal produced is more or less oxidized and the silicon loss from the charge varies from 5 to 15%.

Many inventors have tried to modify such an apparatus in order to avoid the disadvantages thereof. There have been attempts to change the mounting of the tuyeres. A hot blast under pressure has been used, as suggested by Moore of the U. S. A. and also by Piwowarsky in Europe. There has been developed in the U. S. A. a device for continually melting in order to avoid stoppage of the openings, and more recently the silicious refractory linings have been replaced by basic refractory linings. Piwowarsky has proposed a cupola in which a part of the coke is burned in a separate chamber in such a way that all of the carbon may be converted into CO<sub>2</sub>. When a hot blast is used in such cupolas, it is possible to diminish the loss of silicon but the wear and deterioration of the lining is accelerated as a result of the higher temperatures which prevail in the region of the tuyeres, with the result that the operation necessarily remains intermittent.

In spite of the use of hot air the melting continues to take place in an oxidizing atmosphere. The slag has a ratio of CaO to SiO<sub>2</sub> which is less than 1, and it contains a fairly large amount of iron oxide which renders the slag very fusible. The speed of gas flowing through these conventional cupolas is very great because of the relatively small size of these cupolas with respect to the hourly tonnage melted. The temperature of the gas at the outlet of such conventional cupolas is generally quite high, being in the neighborhood of from 700° to 800° C., and this gas generally contains less than 12% of CO.

All systems employed up to the present time are characterized by the fact that the fusion of the charge is unfortunately accompanied by two regrettable phenomena:

1. The oxidation of part of the metallic elements of the charge:



2. The fusion and resulting deterioration of the refractory lining.

These oxidized elements and the molten material of the refractory lining descend with the molten metal and become joined in the slag with neutral elements of the charge, with the result that the operator is not the master of the composition of the slag, as was pointed out above. Several authorities, such as G. Somigli and E. Wittem have regretted this fact. For example, R. Perrin has stated that in a steel foundry the nature of the refractory lining used plays a preponderant and automatic role in the quality of the product obtained because of the nature of the slag which is necessarily greatly affected by the material of the refractory lining.

One of the objects of the present invention is to overcome all of the above serious disadvantages by maintaining a reducing atmosphere within the cupola.

Another object of the present invention is to greatly retard the deterioration of the refractory lining so that the composition of the slag may be controlled in accordance with the material charged into the cupola.

A further object of the present invention is to provide a cupola which is capable of maintaining therein a slag bath of constant depth.

Still another object of the present invention is to provide a means for granulating the slag after it leaves the cupola.

Yet another object of the present invention is to provide a cupola furnace which may also function as a gas producer.

A still further object of the present invention is to provide a cupola furnace capable of producing in a continuous manner a high quality product of constant composition and which may be varied by variation of the compositions of the charge.

An additional object of the present invention is to prevent setting of the slag while it is associated with the cupola.

Still another object of the present invention is to provide a means for draining all molten metal and slag from a cupola when the latter is to be used as a gas producer without stopping up the normal outlet for the molten metal of the cupola.

With the above objects in view the present invention mainly consists of providing a cupola furnace which has an elongated hollow body having a vertical central axis and a bottom wall toward which molten metal and slag move. This hollow body is provided with an inner refractory lining and has a side wall portion adjacent the bottom wall thereof formed with a pair of openings one of which passes through the side wall portion substantially at the level of the bottom wall to lead molten metal from the hollow body and the other of which passes through the side wall portion above this one opening to lead slag from the hollow body. A receiving chamber is connected to the hollow body at the side wall portion thereof and communicates with these openings, this receiving chamber having a slag

discharge spout and a metal discharge spout located below the slag discharge spout. The receiving chamber has a cross-sectional area in a horizontal plane which is substantially smaller than the cross-sectional area of the interior of the hollow body in the same horizontal plane, and the receiving chamber is also provided with a dividing wall extending beneath the lower of the above-mentioned openings and being located between the spouts to separate molten metal and slag from each other. A cooling means is provided to cool the entire outer surface of the hollow body and a gas outlet valve is located at the top of the cupola to maintain the gas pressure therein at a predetermined value so as to maintain a slag bath of predetermined constant depth in the cupola.

With these objects also in view, the present invention mainly comprises means for introducing hot air into a cupola furnace containing an excess of carbon in the charge so as to oxidize said carbon by introduction of said hot air and thus raise the temperature in said cupola furnace and heat the charge therein while maintaining a reducing atmosphere in said cupola furnace, thus melting the metallic oxides in said charge and reducing the same to the corresponding metal; and maintaining in said cupola furnace a slag bath of constant depth through which said molten metal passes so as to cause said metal to react with said slag bath under uniform conditions, thereby obtaining a metal having uniform properties.

The novel features which are considered as characteristic for the invention are set forth in particular in the appended claims. The invention itself, however, as to its construction, together with additional objects and advantages thereof, will be best understood from the following description of specific embodiments when read in connection with the accompanying drawings, in which:

Fig. 1 is an elevational view of a furnace constructed in accordance with the present invention and with parts thereof shown in section, Fig. 1 being taken along line 1—1 of Fig. 3 in the direction of the arrows;

Fig. 2 is a front elevation of the lower part of the cupola of Fig. 1, taken along line 2—2 of Fig. 3 in the direction of the arrows;

Fig. 3 is a plan view of the cupola of Fig. 1 taken along line 3—3 of Fig. 1 in the direction of the arrows;

Fig. 4 is a fragmentary sectional elevation taken along a central diameter of the lower part of the cupola;

Fig. 5 is a sectional view taken along line 5—5 of Fig. 4 in the direction of the arrows;

Fig. 6 is a sectional view taken along line 6—6 of Fig. 5 in the direction of the arrows;

Fig. 7 is a side elevation of a part of the furnace as seen from the right hand side of Fig. 2; and

Fig. 8 is an elevational view of a detail of the cupola illustrated in the above figures.

Referring now to the drawings, it is seen that the cupola of the present invention is provided with a refractory lining 1. Although it is possible to provide the disclosed cupola with various refractory linings, it is preferred to provide the same with a novel refractory lining capable of being applied in situ or capable of being made into bricks which can then be mounted in the interior of the furnace.

Up to the present day it has been necessary

to provide refractory linings having different compositions depending upon the uses for which they were intended. In order to provide a refractory lining which might be suitable for various different uses, several compositions have been proposed, but these compositions either have an extremely low carbon content or no carbon at all.

It is therefore another object of the present invention to provide a novel refractory lining which is particularly suitable for cupola furnaces.

It is an additional object of the present invention to provide a process for forming such novel refractory lining in a cupola furnace.

With the above objects in view the present invention mainly comprises a refractory lining essentially consisting of finely divided particles of carbon, silica, alumina, ferric oxide, calcium oxide and magnesia.

According to the preferred embodiment, the finely divided particles have a size of less than 5 mm. and are present in the proportion of 1 part carbon to 1.4-1.7 parts silica, 0.07-0.11 part alumina, 0.007-0.023 part ferric oxide, 0.003-0.012 part calcium oxide and 0.0010-0.0035 part magnesia. The terms "part" and "parts" as used in the specification and claims refer to the molecular ratio of the substances to each other. The ratio of each of the substances of the refractory lining to each other is by molecules rather than by weight.

The process for producing the refractory lining according to the present invention mainly comprises the steps of homogeneously mixing finely divided particles of carbon, silica, alumina, ferric oxide, calcium oxide and magnesia, heating the thus formed homogeneous mixture under pressure so as to form a substantially solid mass of the finely divided particles, thereby obtaining a refractory lining for furnaces.

In the past refractory linings subjected to extreme conditions, as much thermochemical as mechanical, presented the inconvenience of requiring different compositions for different purposes for which the lining was intended; another inconvenience was the frequent necessity of stopping the operation of the furnace in order to repair the lining which was partially destroyed at the high temperatures of operation of the furnace. This was particularly the case with hot blast cupolas.

Various different compositions have been proposed to remedy these inconveniences. These compositions contain either no carbon at all or very little carbon. Occasionally bricks forming these linings were placed on a bed of bricks made of practically pure carbon. The following table indicates the usual composition of refractory linings which do not contain carbon:

|                                | Percent | Percent | Percent | Percent | Percent |
|--------------------------------|---------|---------|---------|---------|---------|
| SiO <sub>2</sub>               | 51.5    | 55.5    | 58.5    | 81      | 96      |
| Al <sub>2</sub> O <sub>3</sub> | 43      | 37.5    | 34.5    | 16      | 1.55    |
| Fe <sub>2</sub> O <sub>3</sub> | 2.5     | 4.5     | 3       | 1.2     | 0.5     |
| CaO                            | 0.5     | 0.5     | 0.7     | 0.3     | 1.7     |
| MgO                            | 0.6     | 0.5     | 0.5     | 0.5     | 0.05    |
| Misc.                          | 2       | 1.5     | 3       | 1       | 0.3     |

One of the characteristics of the present invention is the uniting in the same refractory composition of carbon with the substances listed above.

One can thus prepare a lining capable of re-

sisting extremely high temperatures as well as being capable of resisting acid and basic slags. These linings are particularly suitable for metallurgical cupolas utilizing hot air, the exterior of which furnace is cooled and which cupolas can function also as a gas producer.

The novel lining used in the cupola of the present invention unites with the conventional elements in such refractory linings a predetermined quantity of carbon. The novel lining is produced by combining with carbon, in a predetermined molecular proportion, other elements which are normally used in refractory linings such as SiO<sub>2</sub>, Al<sub>2</sub>O<sub>3</sub>, Fe<sub>2</sub>O<sub>3</sub>, CaO, and MgO. All of these elements are ground, milled, pulverized or crushed until their grains have a size of less than about 5 mm. A mixture is then formed from these elements, in such quantities that after drying they will be in the refractory lining in the following molecular proportions:

For 1 C:

from 1.4 to 1.7 SiO<sub>2</sub>,  
from 0.07 to 0.11 Al<sub>2</sub>O<sub>3</sub>,  
from 0.007 to 0.025 Fe<sub>2</sub>O<sub>3</sub>,  
from 0.003 to 0.012 CaO, and  
from 0.0010 to 0.0035 MgO.

A characteristic of this novel lining is that after drying the molecular ratio of SiO<sub>2</sub> to Al<sub>2</sub>O<sub>3</sub> is between 12 and 25. To this mixture thus obtained, only sufficient water is added to form a coherent mass, this quantity of water being in the vicinity of 4-8% by weight of the mixture. With such a lining it is possible for a cupola to operate continuously for long periods of time while maintaining a basic slag.

To the mixture obtained above is added a minimum amount of water which is necessary to form a paste which may be tamped or briquetted under pressure into a coherent mass. This quantity of water is preferably about 4-8% by weight by the total weight of the mixture.

It is thus possible to conveniently line in situ or with the help of bricks of the above indicated composition the crucible of the cupola furnaces. The use of the lining according to the present invention is particularly advantageous in the case of hot blast cupolas where the thickness of the lining is less than 150 mm., the lining being utilized to the exclusion of any other auxiliary lining.

With the use of the refractory lining according to the present invention metallurgical cupolas having a continuous flowing of basic slag can function for very long periods of time without interruption. Of course, the lining may be employed for other fusion apparatus, or for filling pockets in the lining through which the slag flows. It is also possible to obtain, by briquetting under pressure, any desired shape or form of refractory bricks which can be heated by any means to 1300° C. or more.

In all cases, the lining presents the advantage of permitting utilization of apparatus lined therewith for a long period of time without deterioration of the lining and without the necessity of repairing fissures therein. Therefore, such linings are particularly advantageous for cupolas according to the present invention.

The proportions given above for the refractory lining according to the present invention are the preferred proportions and it is possible to deviate considerably from the amounts without

greatly diminishing the properties of the refractory lining.

The cupola is provided with a top which normally remains closed, although it is provided with a suitable conduit for carrying away gas, and this conduit is provided, as shown in Fig. 1, with a valve 1' adjacent the top of the cupola to cupola to maintain a constant gas pressure therein. This valve can also be located at some distance below the top, if desired. This gas pressure, produced by the air entering through the tuyères and reacting with the charge in the cupola, completely controls the thickness of the slag bath, as has been proved by experiment. Increasing or decreasing the charge only increases or decreases the rate of slag and metal flow and has no effect on the depth of the slag bath. The charge is placed in the cupola through a pair of doors overlying each other at the top of the cupola, and these doors are never opened simultaneously during operation of the cupola, so that the cupola top is always closed except for the gas outlet valve.

As is shown in Fig. 2, the cupola is provided, not far from its bottom, with a plurality of tuyères which are slidably mounted in cylindrical openings 50, respectively, for axial movement so that the tuyères 51 may be adjusted with the outlet ends thereof located at a predetermined distance from the inner lining 1. By arranging the tuyères so that their inner ends extend inwardly beyond the inner lining 1, the tuyères provide, in their horizontal plane, a concentrated area of combustion which is spaced from the refractory lining so as to greatly retard deterioration thereof. Hot air is supplied to the furnace through the tuyères 51 by means of pipes 52 connected to a common air supply which is heated with the hot gas derived from the cupola. The tuyères 51 are sealed with respect to the openings 50 and the pipes 52 by means of cords of asbestos 53, which enable the tuyères to be shaped conically, as illustrated, so as to act as nozzles. By moving the tuyères in the openings 50 it is possible to expand or contract the concentrated combustion area located therebetween. The tuyères 51 are hollow, as clearly shown in Fig. 2, and they are connected with inlet and outlet pipes for circulating cooling fluid through the tuyères. These inlet and outlet pipes preferably communicate with a tank, or the like (not shown), located above the tuyères so that the fluid therein is under a certain pressure which assures that the tuyères will always be filled with the cooling fluid.

As is shown in Fig. 4, the bottom wall 2 of the cupola is inclined. A pair of opposite discharge openings 3 and 4 are respectively located on opposite sides of the cupola passing through the side walls thereof, the opening 3 being horizontal and located at the highest level of the inclined floor 2, whereas the opening 4 is horizontal and located at the lowest level of the inclined floor 2. When the cupola operates as a furnace for producing molten metal, the opening 4 is plugged and the molten metal flows out through the opening 3 into an outer receiving chamber 55. This opening 3 is fairly long and of a fairly small diameter so that it might become plugged if a special means were not provided to prevent this. Due to its small size and fairly long length, the opening 3 is difficult to unstop. When the melting operations are interrupted, there will always remain within the cupola a residual amount of metal and slag which would plug up the opening

3 were it not for the inclined floor 2 leading down to the discharge opening 4. This latter opening is periodically opened when the melting is interrupted, as for example when the cupola is switched over from use as a melting furnace to use as a gas producer, and the residual molten metal and slag which run out through the opening 4 enables the opening 3 to be maintained clear so that it is almost never necessary to unplug the opening 3.

As is clearly shown in Fig. 4, an inclined opening 5 is provided above the opening 3. Molten metal flows from the interior of the cupola through the opening 3 and down the inclined floor 36 of the receiving chamber 55. Slag flows from the interior of the cupola body through the inclined opening 5 to the interior of the chamber 55 and rests on the molten metal located therein. Thus, the openings 3 and 5 provide separate paths for the metal and slag, respectively.

It will be noted that the cross-sectional area of the chamber 55 in a horizontal plane is much smaller than the cross-sectional area of the cupola in the same horizontal plane. Thus, if it should sometimes happen that there is a variation in the pressure or depth of the slag in the chamber 55, this variation will have almost no effect on the depth of the slag bath within the cupola so that this depth will remain constant in accordance with the gas pressure prevailing in the cupola.

The chamber 55 is provided with a substantially central dividing wall 56 located between the outlet spout 30 for the molten metal and the outlet spout 6 for the slag. It will be noted from Figs. 4-6 that the dividing wall 56 is formed with an opening 32 located below the opening 3 at the lower side of inclined wall 36 to direct molten metal to the upwardly extending opening 33 which communicates with the outlet spout 30.

The top of the chamber 55 is covered by a channel having the cross-section of an inverted U-shape and being provided with a front open end to provide a space 41 where the slag communicates with the outer atmosphere. The molten metal also communicates with the outer atmosphere at the spout 30. The front wall of the chamber 55 is provided with a pair of openings 31 and 35 removably covered by a door 37 mounted on a front plate 40 which covers the entire front of the chamber 55 except for the space 41 and a space 39 located just below the space 41. This space 39 is located opposite the opening 5 so that a rod inserted through the opening 39 may extend into the opening 5 to unplug the same when required. The opening 31 is aligned with the opening 3 to enable the latter to be unplugged when required, and the opening 35 permits the entire chamber 55 to be drained. The top of the chamber is provided with a supporting surface 7 communicating through an opening with the interior of the chamber, as is clearly shown in Fig. 4, so that an oil burner 57, or the like, may be mounted on this support 7 to heat slag within the chamber 55 so as to prevent setting thereof when the slag has a high viscosity. The plate 40 may be removably mounted on the chamber 55 by means of slots through which perforated lugs extend with pins located in these perforations to removably maintain the plate 40 in position, as is clearly shown at 58 in Fig. 2, for example. As is apparent from Fig. 3, these pins are tapered so that the plate 40 may be tightly held in position.

The cupola is cooled over its entire surface by a special cooling means. This cooling means includes a perforated pipe 60 located at the top of the cupola body about the same, as is shown in Fig. 1, and communicating with any source of the cooling water so that this water may flow from the perforations in pipe 60 onto the outer surface of the cupola and down the same. Located about the cupola body at the level of the slag spout 6 and just beneath the tuyères is a gutter 19 which receives the cooling water flowing down the outer surface of the cupola from the pipe 60. A pair of outlet pipes 20 and 21 are connected to the bottom wall of gutter 19 and deliver water from the same to a second gutter 16 located about the cupola at the bottom thereof. Just beneath the gutter 19 there is located a second perforated pipe 28 which extends almost completely about the cupola, this pipe being interrupted at the points where the chamber 55 is joined to the cupola body. This pipe 28 may communicate with the same source of fluid as the pipe 60. The water flowing from perforated pipe 28 moves down the outer surface portion of the cupola located between the gutters 19 and 16 and is collected in the latter.

As is shown in Fig. 4, the gutter 19 extends about the cupola body between the same and the upper part of the chamber 55 so that the water in the gutter 19 cools the upper part of the chamber 55 as well as the cupola portion located adjacent thereto.

As is shown most clearly in Fig. 5, the dividing wall 56 is provided with a space 42. As is shown most clearly in Fig. 2, a conduit 22 communicates with the gutter 19 and has an open end located over this space 42 so that water from the gutter 19 will be directed to this space 42 to fill the same and flow down the outer surface of the chamber 55. A plate 29 extends in an inclined direction, as shown in Figs. 2 and 3, from the space 42 to the gutter 16 so as to prevent water in gutter 16 from splashing into the metal in outlet spout 30.

A special means is provided, as shown in Figs. 3 and 8, for cooling the chamber 55 and cupola at the junctions between the same. This means takes the form of a pair of metal plates 25 and 26 having the same curvature as these junctions, extending downwardly from the lower surface of gutter 19, and being located directly opposite the cupola walls at these junctions. The floor of gutter 19 is provided with a pair of slots 23 and 24 having the same curvature as the plates 25 and the junctions between the cupola and receiving chamber 55 so that water in the gutter 19 will necessarily flow to the narrow spaces between the plates 25 and 26 and these junctions to provide a very effective means for positively cooling the latter so as to effectively prevent excessive strains and cracking at this usually weak point in the cupola construction.

Fixedly mounted on a side wall of the chamber 55 is a box 9 which communicates with a pipe 8 to receive cooling water therefrom, this cooling water for example being derived from the same source which supplies cooling water to the tuyères. The box 9 is traversed by the bottom wall 11' of the slag discharge spout 6, and the box 9 is also traversed by an open top channel 10 having a bottom wall 11'' joined to the box 9 which is provided with an opening located between walls 11' and 11'' to provide a free space into which water may flow from the box 9 down the channel 10 along the floor 11''. Thus, slag 75

falling from the spout 6 and off from the floor 11' will necessarily contact the cooling water flowing down the floor 11'' of channel 10 from space 13 and will be granulated thereby. The 5 slag combined with this water flows down the channel 10 to a downwardly directed pipe 14 which has a closed top and which is opened at the side where it is joined to channel 10 so that the water and slag may fall into the pipe 14 and fall down the same to a pit located beneath the cupola. The pipe 14 is also open on one side thereof at the part where it crosses the gutter 16, and the latter is provided with an extension 15 and channel 17 having an inclined bottom 18 10 and communicating with the interior of pipe 14 so that the water from gutter 16 which includes the water from pipes 20 and 21 combines with the water and slag of channel 10 in the pipe 14 to move down the pipe 14 to the collection pit.

Thus, a very effective means is provided for cooling the entire outer surface of the cupola so as to prevent, as much as possible, deterioration of the lining 1, and the location of the inner ends of the tuyères also contributes to this result, as explained above, so that with the above described cupola the deterioration of the refractory lining 1 will be very greatly retarded and the slag composition will not be contaminated by the material of the refractory lining. In this 25 way the composition of the slag may be maintained constant in accordance with the materials charged into the cupola.

The present invention is based on the known fact that if one progressively increases the metallic elements in the charge of a gas producer one obtains an apparatus which functions as a cupola and produces metal as its principal product and gas as its by-product.

One of the more important aims of the present invention is to provide a process and cupola which enables an industrial foundry iron usable after the first melt to be produced from scrap iron or a mixture of scrap with old iron.

The characteristic fundamentals of the process 45 of the present invention are the following:

1. The melting takes place in a reducing atmosphere.
2. The droplets of metal pass through a high temperature slag bath of constant depth and substantially constant composition.
3. The furnace can operate either as a cupola or a gas producer.

Each of these three points will now be separately described.

1. Melting in a reducing atmosphere, that is to say in an atmosphere such that the elements of the charge such as silicon, iron and manganese do not have a tendency to become oxidized.

According to the classical equations



In principle, in the immediate neighborhood of the tuyères of a conventional cupola, where the concentration of oxygen is greatest and the temperature is lowest, the combustion takes place according to reaction 1. Reaction 2 takes place only higher up, above the tuyères.

According to the present invention, an excess of carbon is utilized in the charge of the cupola

## 11

in relation to the normal fusion requirements of the furnace. Heated air is supplied through the tuyères and the oxygen in the heated air reacts with the carbon according to Equation 1 to produce carbon dioxide and calories which raise the temperature in the cupola. A very high temperature of higher than 1600° C. is provided at the outlet end of the tuyères. At this high temperature the carbon dioxide produced reacts with the excess coke according to Equation 2 to form carbon monoxide. The carbon monoxide forms a reducing atmosphere at very high temperature. The metal oxides in the charge melt in this reducing atmosphere and are reduced while passing therethrough to form the corresponding reduced metal.

The amount of carbon which is included in the charge of the cupola furnace is such that there will always be an excess of carbon as compared to the amount of oxygen which is introduced into the furnace. The factors which control the amount of excess are: the speed of flow of air introduced into the cupola, the amount of air and the amount of carbon. According to the process of the present invention there is always sufficient carbon in the cupola, to constitute an excess when compared to the amount of oxygen that enters the cupola. This excess of carbon, coke being preferred because of its rich carbon content, is the basis for the reducing atmosphere which is at all times present in the cupola.

The process of the present invention is not so much concerned with an efficient use of the combustible material as it is with the production of a high quality metal, and therefore the aim is to produce a reducing atmosphere within the cupola while more or less neglecting the factor of fuel consumption, since the principal purpose of the cupola is to produce a cast iron which is of a high quality, and in order to produce such a high quality cast iron an oxidizing atmosphere must at all times be avoided within the cupola.

In order to obtain this reducing atmosphere, the fluid containing oxygen is introduced into the cupola at a relatively high temperature of between 400 to 600° C. This temperature of the fluid may be obtained by reheating it before it passes through the tuyères. Also the charge located within the furnace preferably has a carbon content of from 15 to 20% which is an excess in relation to the normal requirements of the furnace. The fluid containing oxygen is introduced into the cupola at a speed of from 80 to 100 meters per second. The pressure of the fluid introduced into the cupola in accordance with the present invention is much higher than the pressure used in conventional blast cupolas. In a cupola producing two tons of metal per hour, this pressure would be 60 cm. of water above atmospheric pressure as compared with 25 cm. of water above atmospheric pressure used in a conventional blast cupola.

The results produced by the above described process are that an essentially reducing atmosphere is obtained within the cupola due to the high percentage of carbon, the high heat of the fluid containing oxygen and the high speed with which this fluid is introduced. Also this high speed of introduction of the oxygen-containing fluid results in the fire being maintained within the cupola at about the center thereof, and the CO<sub>2</sub> combines with the carbon to produce CO in a very rapid manner. At a few centimeters

## 12

above the level of the tuyères, the gas is composed almost entirely of CO. As a result of the combustion of carbon into CO a great amount of heat is produced which is in the neighborhood of 2800 calories per kilogram of carbon and this great heat is utilized in the hot blast cupola to assure the melting of the iron charge and the formation of slag. The extremely high temperature within the cupola results in a relatively easy formation of slag which is free of iron oxide and which has between 1.4 and 1.5 times as much CaO as SiO<sub>2</sub>. This slag is much less fusible than slag produced in conventional cupolas. The resulting high temperature in this central melting zone can easily reach a temperature of 1800° C. and can be carried up to 2000° C. by the use of additional oxygen. Because of the relatively large dimension of the interior of the cupola with respect to the cross-sectional area of the tuyères, the gas within the cupola slowly rises and therefore leaves the cupola at the outlet thereof at a relatively low temperature which is substantially below 700° C. This gas which is produced in the cupola has a CO content which is about seven times the CO<sub>2</sub> content thereof.

The introduction of the heated air into the cupola at the relatively high speed of 80-100 meters per second results in the creation of a reducing atmosphere at a very high temperature, i. e. about 1800° C. in the region where the air is introduced into the cupola. The high temperature zone is concentrated about the zone of introduction of heated air which is the fusion zone of the cupola.

Furthermore, it has been found that the introduction of the heated air into the cupola at high speeds, namely 80-100 meters per second, results in a rapid rise in temperature and yields a much faster reaction due to the concentration of the hot reducing atmosphere about the reaction zone of the cupola.

The introduction of heated air into the cupola at speeds substantially below 80 meters per second results in a lower temperature than is produced with the introduction of air at higher speeds, i. e. about 1600° C. It has also been found that there is a great heat loss from around the reaction zone in the cupola due to the heat radiation therefrom. Therefore, in such case, not only is the reaction zone at a lower temperature but the high temperature is less concentrated and therefore the temperature in the cupola at a distance above the reaction zone is higher if the hot air is introduced slowly than is the case if the hot air is introduced rapidly.

For example, assuming the temperature in the zone of introduction of the heated air to be 1800° C. where the heated air is rapidly introduced at a rate of 80-100 meters per second according to the present invention, the temperature rapidly decreases above this zone so that at a relatively short distance therefrom the temperature in the cupola is relatively low, i. e. about 800° C. If the heated air is introduced at a much slower rate the temperature about the zone of introduction of the heated air is lower, i. e. about 1600° C., and at the same distance from this zone as in the above case, wherein the temperature in the cupola is down to about 800° C., the temperature in the cupola at the same distance is still quite high, i. e. about 1500° C.

The amount of air required for the reaction is the same whether or not the speed of introduction of air into the cupola is rapid or slow. Therefore, if the speed of introduction of the heated air into the cupola is substantially below 80 meters per second, it is necessary to provide the cupola with larger tuyères in order to allow for a sufficient amount of air to enter the cupola. It is thus possible by the rapid introduction of the heated air into the cupola to utilize smaller tuyères which, therefore, have the effect of creating a more concentrated zone of oxidation of the carbon in the charge and therefore a more concentrated fusion zone.

The higher speed of reaction resulting from the use of high speeds of introduction of heated air into the cupola has been found to be very beneficial, the yield having been found to be directly proportional to the speed of the reaction.

The oxidation of the carbon, either directly to carbon monoxide or first to carbon dioxide with subsequent reduction according to Equation 2 above, to carbon monoxide, results in an overall exothermic process which raises the temperature in the cupola furnace to an extremely high temperature for such cupolas, namely 1550-1600° C. The high temperature and the reducing atmosphere of the cupola result in the reduction of the metallic oxides to the corresponding reduced metals. The reducing atmosphere at high temperature also results in a reduction of the metallic sulfides by transfer of the sulfide from the iron to calcium or other similar metals. This shall be more clearly explained later.

Another extremely important advantage of the process of the present invention is the maintaining of a slag bath having constant depth and substantially constant composition. Since the reduced metal passes through the slag bath where it reacts to be further reduced and to combine with other elements such as carbon to form alloys, the importance of maintaining a slag bath of constant depth and substantially constant composition is obviously great. If the depth of the slag bath and/or the composition were to vary during the operation of the cupola furnace, the metal droplets which pass therethrough would not react uniformly and the product produced would therefore not have uniform properties.

As explained elsewhere in the application, the depth of the slag bath is maintained constant by the use of the special apparatus of the present invention. Further, the composition of the slag bath normally varies due to the melting and decomposition of the refractory lining of the cupola furnace which mixes with the slag bath. The present invention by providing for cooling of the wall of the cupola furnace during the operation of the same prevents the melting and decomposition of the refractory lining and thereby prevents the contamination of the slag bath with the materials of the refractory. This results in a slag bath of substantially constant composition.

The composition of the slag bath is further maintained constant by the apparatus of the present invention which provides for the introduction of the heated air in an area spaced from the wall of the cupola furnace. This aids in preventing the decomposition of the refractory lining of the surface and is therefore a further aid in maintaining a constant composition of the slag bath.

According to the invention air at a tempera-

ture of approximately 500° C. is supplied through the tuyères, and the tuyères are disposed in such a way as to add to the temperature at their outlet ends so as to thus produce the endothermic Reaction 2. The gas producing zone can be considered as the gas producing zone of a gas producer cooled by the molten metal which passes from the top to the bottom. The metal melts in a reducing atmosphere of carbon monoxide, and it moves downwardly in the form of droplets and the FeO, which has for example been charged in the form of rust and which is dissolved into the iron, is reduced in passing through this superheated reducing zone.

15 The iron, in the proportion that it is melted, absorbs carbon which is not burned in passing the tuyères.

It is a well known fact that at a temperature of 1803° C., oxygen has a much greater affinity for carbon than for silicon so that at this temperature it is absolutely impossible for silicon to unite with oxygen and become silica. On the contrary, the reverse takes place, and the silica in the charge is reduced to silicon by the carbon or CO. With the process of the present invention it is possible to obtain 2.5% silicon at the outlet of the cupola when the original charge contained 2.2% silicon.

Even if the scrap iron charged is very highly oxidized, the FeO content of the slag obtained never exceeds 0.8% which shows that the slag never contains all of the iron content of the ashes in the coke charged.

35 In a classical cupola, the attempt is always to burn as much carbon as possible into CO<sub>2</sub>, which prevents working in a very high temperature, with the result that the conditions are those that produce a zone where silicon, manganese and iron are necessarily oxidized.

40 Melting in a reducing atmosphere according to the present invention produces moreover two additional advantages:

(a) No metallic elements are lost to the slag. H. Jungbluth has established that the loss of 45 iron in a cupola is proportional to the ratio of



50 With the present invention this ratio is very low, and this has an important economical advantage if one considers that those elements which are most easily oxidized obviously are those whose reduction is most difficult, and as a consequence these elements are the costliest since they require an extremely high gross weight to produce 1000 kg. of useful metal in the furnace.

(b) The composition of slag is not, as in the 60 conventional cupola, modified by the oxidized elements in the zone of fusion in a way which cannot be controlled. It is known that in a conventional apparatus, where the zone of fusion is oxidizing, numerous uncontrollable factors intervene in the process, such as pressure and humidity of the air, for example, to slightly modify the atmosphere of the furnace so that it will become oxidizing for one element or reducing for another element or vice versa. With the process of the present invention, however, such a changeable zone of fusion is completely avoided, and the reactions always take place in a reducing atmosphere.

70 2. The molten metal droplets pass through a

layer of slag whose composition and thickness is constant and whose temperature is very high.

It is relatively unimportant that an equilibrium of reaction cannot take place because of the small length of time during which the droplets of metal pass through the slag. Substantially the same result can be obtained if constant controllable reactions can be produced during the time that the molten metal droplets pass through the slag, and so it is sufficient if the layer of slag has a constant thickness. As a result of this feature, which is obtained by continuous drawing off of the slag from the furnace as it is being produced therein, it is possible to maintain in the interior of the furnace a slag having a thickness of the order of 300 mm., whereas with a conventional cupola one can be satisfied with an extremely simple device since the only objective is to provide a mechanical separation of metal from slag.

In order to maintain the composition of the slag constant, it is necessary to avoid contamination of the slag with the material of the refractory lining, and this is done by the above-described very efficient cooling of the wall of the furnace as well as by extending the tuyères to a point within the furnace which is beyond the inner surface thereof so that the combustion area defined by the outlet ends of the tuyères is located away from the inner lining of the furnace. It is true that this strong cooling of the furnace is very costly in calories, but from a metallurgical point of view it is indispensable if the operator is to be the master of the composition of the slag.

Finally, the high temperature which obtains in the gasification zone gives the slag a very high temperature.

According to known principles it is most desirable that the molten metal have the greatest opportunity to react with the slag in order that desirable elements in the slag may be absorbed into the metal and undesirable elements may be absorbed into the slag. The degree to which these desirable reactions take place increases with an increase in temperature, and according to the present invention the cupola operates at a very high temperature. The degree to which these reactions take place also increases with an increase in the surface contact between the metal and slag, and if a comparison is made between the cupola of the present invention and a hearth furnace such as the Martin furnace, or an electric furnace, it will be seen that process of the invention where droplets of metal move through the slag produces at least one hundred times greater surface contact between the metal and the slag.

3. From a thermal point of view, the cupola can be considered as a combination cupola and gas producer.

In conventional processes the aim is to burn in the cupola as much carbon as possible into  $\text{CO}_2$ .

The thermal balance of the process of the present invention is the following:

For 100 calories of coke:

- 26.5 are used to produce molten metal,
- 54 are expended in the form of a gas which may be used for various purposes,
- 1.5 are lost to the slag,
- 10.5 are lost to the cooling water, and
- 7.5 are lost in reheating the combustion air.

70  
75

It is thus possible to combine into the single apparatus of the present invention two devices: a cupola which utilizes 80 kgs. of coke of 7000 calories to melt a ton of metal and a gas producer which gasifies at the same time, without loss, 9.5 kgs. of the same combustible material.

The reduced gas is produced at the rate of 100 kg. per ton of metal for a charge which carries 170 kg. This gas contains 24% CO and 4%  $\text{CO}_2$ .

10 As a comparison there is shown herewith a table of the different types of charges necessary to produce the same metal with the new process and with a conventional cupola.

15

|                                  |         | New Cupola | Conventional Cupola |
|----------------------------------|---------|------------|---------------------|
|                                  | Percent | Percent    | Percent             |
| 20 (a) metallic charge:          |         |            |                     |
| Old Iron.....                    | 50      | 35         |                     |
| Steel.....                       | 43      |            |                     |
| Iron Alloys at 25%               | 7       |            |                     |
| Pig Iron semi-phos. at 3-3.5% Si |         | 50         |                     |
| Waste.....                       |         | 15         |                     |
|                                  | 100     | 100        |                     |
| 25 (b) slag lime.....            | 5 to 8  | 5 to 8     |                     |
| (c) combustible material:        |         |            |                     |
| Coke.....                        | 17      | 13         |                     |
| Ignition Coke.....               | 0.6     | 1.5        |                     |

30

The excessive consumption of combustible material in the new cupola under normal circumstances is evident from this table, but this excessive consumption is largely compensated by the fact that the conventional cupola requires frequent interruptions for repairs, etc. The quantities of combustible material necessary for fusion vary between the following limits:

40 11% of coke having 10% of ashes with a charge of 100% pig iron; and

24% of coke having 10% of ashes with a charge of 100% scrap steel.

For these charges it is necessary to provide about 1000 cubic meters of air for each ton of molten metal.

45 With the apparatus and process of the present invention, when the melting of metal is interrupted the cupola can continue to function as a gas producer. After an interruption of eight hours it is necessary to charge 300-450 kgs. of coke to resume melting of metal; after an interruption of 30 hours 600-700 kgs. of coke would be required.

50 Experience has shown cupolas according to the present invention can be constructed for any desired production capacity, i. e. 5-20 tons per hour and more.

55 By way of example the constructive characteristics of a new cupola having a capacity of 5 tons per hour are the following:

Its capacity is in the neighborhood of 5 tons per hour; the diameter between tuyères is about 850 mm.; its exterior is cooled by water flowing down the same; the tuyères are independently cooled; the top is closed; 35% of the gas is sent to an air reheater, the rest being used for other needs of the foundry.

The air is reheated by passage through three phases of exteriorly heated tubes, this heating being done by the combustion of gas from the cupola. A filter is placed between the cupola and air reheater to retain the larger impurities in the air.

A comparison of the cupola furnace and the process of the present invention as compared to the known cupola furnaces shows the following:

|                         | Normal cold air cupola | Hot air cupola according to Whiting-Griffin-Piwowsky | Cupola according to the present invention |
|-------------------------|------------------------|------------------------------------------------------|-------------------------------------------|
| Coke                    | (10% ashes) 100 kg     | (10% ashes) 60-80 kg                                 | (15% ashes) 200 kg                        |
| Carbon per ton of metal | 80 kg                  | 65 kg                                                | 180 kg                                    |
| Slag per ton of metal   | 60 kg                  | 40 kg                                                | 130 kg                                    |
| Gas Produced:           |                        |                                                      |                                           |
| (1) $\text{CO}_2$       | 15%                    |                                                      | 2-8%                                      |
| (2) $\text{O}_2$        | 1.5%                   |                                                      |                                           |
| (3) $\text{CO}$         | 5%                     |                                                      |                                           |
| Calories                | 200 kcal               | 900-1,000 kcal                                       | 1,550-1,600 kcal                          |
| Temperature of slag     | 1,350° C               | 1,400-1,500° C                                       | 1,550-1,600° C                            |
| Analysis of slag:       |                        |                                                      |                                           |
| (1) $\text{SiO}_2$      | 40%                    |                                                      | 30%                                       |
| (2) $\text{CaO}$        | 28%                    |                                                      | 50%                                       |
| (3) $\text{FeO}$        | 4-5%                   |                                                      | <0.3                                      |
| Working                 | oxidation              | oxidation                                            | extremely reductive                       |
| Carbon or schist        |                        |                                                      | 50 kg. having 70% ashes                   |
| Limestone               | 6 kg                   | 4 kg                                                 | 130 kg                                    |
| New pig iron            | 300 kg                 | 300 kg                                               |                                           |
| Old pig iron            | 700 kg                 | 700 kg                                               |                                           |
| $\text{FeSi}$ (10%)     |                        |                                                      |                                           |
| Scrap iron              |                        |                                                      | 1,000 kg                                  |

The technical possibilities of a cupola according to the invention are:

It is possible to obtain a metal having properties very different from those which are charged because the latter after melting pass in a reducing atmosphere of very high temperature and then into an abundant slag which also has a very high temperature.

Moreover, the only constituents in the slag are obtained from the charge at the top of the furnace. The slag is not contaminated by the elements of the refractory lining. The height of the slag, as well as other factors, are maintained constant to produce internal equilibrium in the apparatus.

It is possible to obtain slags which have a low degree of fluidity and which at the temperatures of conventional cupolas would result in stoppage of passageways and would be impossible to empty.

As a result to these characteristics it is possible to carry out a series of metallurgical operations which produce a final metal product whose analysis depends on the composition of the slag which intervenes in accordance with the laws of chemical equilibrium.

By way of example, it is possible also

(a) To obtain a hematite metal of low sulfur from scrap steel;

(b) To obtain highly carbonized metal from a slightly carburized charge;

(c) To obtain a metal which is highly resistant to the heat or wear which could up to the present time be obtained only from an electric furnace;

(d) To obtain products of different types from the same charges or from a series of different charges by combining various materials with the metal leaving the cupola, this combination being very easy because of the high temperature of the metal as it leaves the cupola.

The apparatus of the present invention is distinguished from the apparatus of conventional hot blast cupolas, in that in the latter there is a constant striving to obtain two objects:

(a) Diminution of coke consumption, and

(b) The use of coke of poor quality.

In accordance with the present invention the operations take place

(a) At extremely high temperatures and in a highly concentrated zone of fusion,

(b) In a highly reducing atmosphere.

Whatever metal is obtained with the process and apparatus of the present invention, it distinguishes from metals made from other apparatus by

(a) A superior flowability as compared to a product produced with the same charge in a conventional cupola,

(b) A less pronounced propensity to tempering as compared to a product produced with the same charge in a conventional cupola.

As a result of the reducing atmosphere which obtains in the cupola of the present invention, the loss of iron is almost completely suppressed. There is actually less iron and manganese in the slag of the present invention than in the ashes of combustion.

The charge used in the process and apparatus of the present invention can include oxidized metals. By varying the temperatures of the air introduced into the cupola and by varying the quantity and quality of combustible material and the quantity and composition of the slag, one can voluntarily control the carbon content of the metal produced. It is thus possible to produce a metal having 3.4% of carbon from a charge of 100% steel, and one can also produce a slightly carbonized metal from a highly carbonized charge.

The phosphorus introduced in the form of phosphorized scrap metal or in the form of phosphates passes completely into the molten metal.

The silicon can be introduced in the form of ferro-silicon or old silicious iron.

In a case where there is little silicon introduced in the charge, it is possible to find all of the silicon of the charge in the metal produced.

The sulfur content can be greatly reduced by controlling the slag.

On the subject of sulfur content, an example is given herewith of the application of the new apparatus to the production of a de-sulfurized product.

Sir Charles Goodeve and J. Pearson have recently written that in order to free iron from sulfur it is necessary to place it in intimate contact with a phase in which the sulfur potential is of a low value and which besides possesses a sufficient absorption capacity; moreover one can lower the sulfur potential by a phase which dissolves sulfur and is composed of an appropriate solvent added to other elements such as the alumino-silicates of calcium which are the least expensive good solvents.

The de-sulfurizing equations can be described as



Then in the midst of the slag:



Finally,



We have seen that the basic principle of the invention is to melt in a reducing atmosphere. The cited authors emphasize that the capacity of a basic slag can be one hundred times greater or advantageous with respect to sulfur in a blast furnace than the same slag under the oxidizing conditions which are produced in a Martin furnace, for example. The atmosphere in the cupola of the present invention closely approaches that of a blast furnace. R. Rocca, N. J. Grant, and J. Chipman have all demonstrated that the degree to which de-sulfurizing takes place will be increased as the quantity of FeO in the slag is decreased.

The amount of FeO in the slag obtained in the present invention is much lower than the critical content of 2% cited by the above authorities since in the slag of the present invention where the apparatus and process is practiced industrially, the FeO content never exceeds 0.8%. It is interesting to note that it is the extremely high FeO content in the slag of conventional cupolas which prevents success in the de-sulfurizing by calcium carbide.

One might think that the two necessary conditions of good de-sulfurizing, that is, the basic slag and a reducing atmosphere, are independent of each other. This is not the case. In effect, in an oxidizing atmosphere, the basic slag is acidified by the silica produced from the oxidation of the silicon in the charge.

Equation 5 shows that carbon is necessary to eliminate the FeO produced by Reaction 4. In a reducing atmosphere and at a high temperature the molten metal becomes rapidly saturated with carbon and as a result of the present invention this latter element is present in a sufficient quantity in each droplet of metal to assure the displacement of equilibrium to the right.

With the process of the present invention the reactions between the metal and slag take place, with respect to de-sulfurization, under very favorable circumstances as much with respect to temperature as with respect to surface contact.

E. Whitten has indicated the importance of high temperature in de-sulfurization. A high temperature promotes separation of sulfur from iron.

Finally, G. Derge, W. O. Philbrook and Kenneth M. Goldman have shown that the speed with which this separation takes place depends to a great measure on the surface of contact between metal and slag, and it has been shown that this surface is at least one hundred times greater in a cupola than in a crucible or electric furnace.

Finally there is presented herewith data relative to a normal process in a cupola of the present invention.

| Silicon charged                                          | 2.10% | 2.37% | 2.32% | 2.14% |
|----------------------------------------------------------|-------|-------|-------|-------|
| Analysis of Metal:                                       |       |       |       |       |
| Silicon..... percent                                     | 2.35  | 2.43  | 2.31  | 2.13  |
| manganese..... do                                        | 0.42  | 0.56  | 0.46  | 0.50  |
| phosphorus..... do                                       | 0.84  | 0.61  | 0.78  | 0.55  |
| carbon (total)..... do                                   | 3.455 | 3.59  | 3.59  | 3.63  |
| sulfur..... do                                           | 0.083 | 0.05  | 0.058 | 0.067 |
| Temperature of the melt..... °C                          | 1,550 | 1,524 | 1,514 | 1,516 |
| Analysis of slag:                                        |       |       |       |       |
| SiO <sub>2</sub> ..... percent                           | 39.8  | 34    | 37.05 | 35.3  |
| CaO..... do                                              | 43.7  | 44.9  | 46.9  | 44.1  |
| Al <sub>2</sub> O <sub>3</sub> ..... do                  | 12.2  | 15.87 | 10.76 | 15.17 |
| FeO..... do                                              | 0.707 | 0.82  | 0.73  | 0.74  |
| MnO..... do                                              | 0.801 | 0.45  | 0.86  | 0.76  |
| CaS..... do                                              | 2.295 | 3.69  | 2.93  | 3.44  |
| S..... do                                                | 1.02  | 1.64  | 1.32  | 1.48  |
| Temperature of the air..... °C                           | 480   | 502   | 549   | 483   |
| Pressure of the air (mm. of water above atmosphere)..... | 754   | 720   | 755   | 758   |
| Temperature of Gas at the top outlet..... °C             | 334   | 393   | 372   | 372   |

## PROPERTIES OF METAL OBTAINED

The molten metal obtained directly from the cupola is very hot (over 1500° C.) and for a metal of the same composition and temperature produced by an ordinary cupola, it has superior flowing qualities and a lesser propensity to tempering and it is possible to very easily combine this metal with other elements inserted into the molten metal.

## (a) Iron for centrifugal cast pipes

To produce this type of iron in a conventional cupola one cannot include steel in the charge if one wishes to avoid reheating of the pipe, and besides one cannot use less than 60% of pig iron.

With the present invention however this same iron can be produced from a charge having only scrap steel and iron.

## (b) Iron having high mechanical resistance

For this iron the standard charge has the following composition:

|                                                              | Per cent     |
|--------------------------------------------------------------|--------------|
| 1. Metals charged:                                           |              |
| Steel                                                        | 85 to 80     |
| Iron alloy having up to 10% Si                               | 15 to 20     |
|                                                              | 100 100      |
| 2. Lime                                                      | 5 to 8       |
| 3. Combustibles (coke)                                       | 15 to 17     |
| which corresponds to a chemical composition of molten metal: |              |
| C                                                            | 2.8 to 3.2   |
| Si                                                           | 1.8 to 2.3   |
| Mn                                                           | 0.5 to 0.8   |
| P                                                            | 0.05 to 0.1  |
| S                                                            | 0.05 to 0.08 |

## MECHANICAL CHARACTERISTIC OF IRON HAVING A HIGH MECHANICAL RESISTANCE

From a 100% steel and iron alloy charge and after combining the molten product with 0.2% of silicocalcium and 0.5% of calcichrome, there is produced a product having a resistance to bending of 56.6 kgs./cm.<sup>2</sup> for a deflection of 9 mm. in a bar 300 mm. long and having a diameter of 0.600 mm. between supports

Resistance to traction: 42.1 kgs./cm.<sup>2</sup>

From 80-85% steel and iron alloy there is produced a shear resistance of 30-40 kgs./cm.<sup>2</sup>.

The Brinell hardness varies in general from 190 to 250 according to the content of carbon and silicon in the molten metal. The hardness varies little over a given thickness.

An examination of a micrograph before etching shows a very fine graphite uniformly distributed. After etching it may be seen that the texture is essentially perlitic.

## (c) Refractory iron (high resistance to heat)

An iron produced from 100% steel and ferro silicon and to which 0.8% of Cr has been added in the molten product, can be used without risk of expansion up to 800° C.

It will be understood that each of the elements described above, or two or more together, may also find a useful application in other types of cupola furnace and process for operating the same differing from the types described above.

What is claimed as new and desired to be secured by Letters Patent is:

1. A cupola furnace, comprising, in combination, an elongated hollow body having a vertical

central axis, a closed top and a bottom wall toward which molten metal and slag move, said hollow body having an inner refractory lining and having a side wall portion adjacent said bottom wall thereof formed with a pair of openings, one of which passes through said side wall portion substantially at the level of said bottom wall to lead molten metal from said hollow body and the other of which passes through said side wall portion above said one opening to lead slag from said hollow body; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; and cooling means associated with the outer surface of said hollow body for cooling the same over substantially the entire outer surface thereof.

2. A cupola furnace, comprising, in combination, an elongated hollow body having a vertical central axis, a closed top and a bottom wall toward which molten metal and slag move, said hollow body having an inner refractory lining and having a side wall portion adjacent said bottom wall thereof formed with a pair of openings, one of which passes through said side wall portion substantially at the level of said bottom wall to lead molten metal from said hollow body and the other of which passes through said side wall portion above said one opening to lead slag from said hollow body; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; cooling means associated with the outer surface of said hollow body for cooling the same over substantially the entire outer surface thereof; and a plurality of tuyères mounted on said hollow body in a horizontal plane substantially at the level of said discharge spout.

3. A cupola furnace, comprising, in combination, an elongated hollow body having a vertical central axis, a closed top and a bottom wall toward which molten metal and slag move, said hollow body having an inner refractory lining and having a side wall portion adjacent said bottom wall thereof formed with a pair of openings, one of which passes through said side wall portion substantially at the level of said bottom wall to lead molten metal from said hollow body

and the other of which passes through said side wall portion above said one opening to lead slag from said hollow body; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; cooling means associated with the outer surface of said hollow body for cooling the same over substantially the entire outer surface thereof; and a plurality of tuyères mounted on said hollow body in a horizontal plane substantially at the level of said discharge spout, said tuyères extending into said hollow body beyond said inner refractory lining thereof to provide a combustion area in the horizontal plane of said tuyères which is spaced from said refractory lining.

4. A cupola furnace, comprising, in combination, an elongated hollow body having a vertical central axis, a closed top and a bottom wall toward which molten metal and slag move, said hollow body having an inner refractory lining and having a side wall portion adjacent said bottom wall thereof formed with a pair of openings, one of which passes through said side wall portion substantially at the level of said bottom wall to lead molten metal from said hollow body and the other of which passes through said side wall portion above said one opening to lead slag from said hollow body; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; cooling means associated with the outer surface of said hollow body for cooling the same over substantially the entire outer surface thereof; and a plurality of tuyères mounted on said hollow body in a horizontal plane substantially at the level of said discharge spout, said tuyères extending into said hollow body beyond said inner refractory lining thereof to provide a combustion area in the horizontal plane of said tuyères which is spaced from said refractory lining, and said tuyères being adjustably mounted on said hollow body for movement toward and away from said central axis thereof so that the size of said combustion area may be varied.

5. A cupola furnace, comprising, in combination, an elongated hollow body having a vertical central axis, a closed top and a bottom wall

toward which molten metal and slag move, said hollow body having an inner refractory lining and having a side wall portion adjacent said bottom wall thereof formed with a pair of openings, one of which passes through said side wall portion substantially at the level of said bottom wall to lead molten metal from said hollow body and the other of which passes through said side wall portion above said one opening to lead slag from said hollow body; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; cooling means associated with the outer surface of said hollow body for cooling the same over substantially the entire outer surface thereof; and a plurality of tuyères mounted on said hollow body in a horizontal plane substantially at the level of said discharge spout, said tuyères being hollow so that they may be cooled by a cooling fluid located therein.

6. A cupola furnace, comprising, in combination, an elongated hollow body having a vertical central axis, a closed top and a bottom wall toward which molten metal and slag move, said hollow body having an inner refractory lining and having a side wall portion adjacent said bottom wall thereof formed with a pair of openings, one of which passes through said side wall portion substantially at the level of said bottom wall to lead molten metal from said hollow body and the other of which passes through said side wall portion above said one opening to lead slag from said hollow body, said one opening being substantially horizontal and said other opening being inclined upwardly from the interior of said hollow body; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; and cooling means associated with the outer surface of said hollow body for cooling the same over substantially the entire outer surface thereof.

7. A cupola furnace, comprising, in combination, an elongated hollow body having a vertical central axis, a closed top and a bottom wall toward which molten metal and slag move, said hollow body having an inner refractory lining and having a side wall portion adjacent said bottom wall thereof formed with a pair of openings, one of which passes through said side wall

70

65

60

55

40

25

10

20

15

5

30

25

20

15

10

5

35

30

25

20

15

10

5

portion substantially at the level of said bottom wall to lead molten metal from said hollow body and the other of which passes through said side wall portion above said one opening to lead slag from said hollow body, said bottom wall being inclined downwardly from said one opening and said hollow body being formed with an additional opening passing through the side wall thereof and communicating with the lowermost part of said inclined bottom wall; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; and cooling means associated with the outer surface of said hollow body for cooling the same over substantially the entire surface thereof.

8. A cupola furnace, comprising, in combination, an elongated hollow body having a vertical central axis, a closed top and a bottom wall toward which molten metal and slag move, said hollow body having an inner refractory lining and having a side wall portion adjacent said bottom wall thereof formed with a pair of openings, one of which passes through said side wall portion substantially at the level of said bottom wall to lead molten metal from said hollow body and the other of which passes through said side wall portion above said one opening to lead slag from said hollow body, said bottom wall being inclined downwardly from said one opening and said hollow body being formed with an additional substantially horizontal opening passing through the side wall thereof and communicating with the lowermost part of said inclined bottom wall; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; and cooling means associated with the outer surface of said hollow body for cooling the same over substantially the entire surface thereof.

9. A cupola furnace, comprising, in combination, an elongated hollow body having a vertical central axis, a closed top and a bottom wall toward which molten metal and slag move, said hollow body having an inner refractory lining and having a side wall portion adjacent said bottom wall thereof formed with a pair of openings, one of which passes through said side wall

75

portion substantially at the level of said bottom wall to lead molten metal from said hollow body and the other of which passes through said side wall portion above said one opening to lead slag from said hollow body; a receiving chamber connected to said hollow body at said side wall portion thereof and communicating with said openings, said receiving chamber having a slag discharge spout and a metal discharge spout located below said slag discharge spout and said receiving chamber having a cross-sectional area in a horizontal plane which is substantially smaller than the cross-sectional area of the interior of said hollow body in the same horizontal plane, said receiving chamber also having a dividing wall extending beneath said one opening and being located between said spouts to separate molten metal and slag from each other; gas outlet valve means located adjacent said top of said hollow body to maintain therein a slag bath of constant depth; cooling means associated with the outer surface of said hollow body for cooling the same over substantially the entire surface thereof; and support means located on said chamber adjacent an upper part thereof to support a heater for heating slag in said receiving chamber so as to prevent setting of slag in said receiving chamber.

10. A cupola furnace as defined in claim 2 and wherein said cooling means comprises a first perforated pipe located about said hollow body adjacent the top thereof for spraying cooling water on the outer surface of said hollow body, a first gutter located about said hollow body substantially at the level of said tuyères for receiving cooling water from said first pipe, a second perforated pipe located about said cupola just beneath said first gutter for spraying cooling water on said cupola below said first gutter, a conduit communicating with said first gutter and having an open end located adjacent said

receiving chamber for guiding cooling water from said first gutter onto said chamber, and a second gutter located about said cupola at the bottom thereof for receiving cooling water from said conduit and second perforated pipe.

11. A cupola furnace as defined in claim 10  
and wherein metal plates are mounted close to  
the outer surface of said hollow body respectively  
at the junctions thereof with said receiving  
10 chamber and wherein said first gutter is formed  
with slits located over said metal plates between  
the same and said hollow body and conforming  
to the shape thereof to direct liquid from said  
first gutter onto said hollow body between the  
15 same and said metal plates so as to cool said  
hollow body and receiving chamber at said  
junctions.

12. A copula as defined in claim 1 and wherein said receiving chamber is formed with a pair of passages respectively aligned with said openings to permit rods to be inserted through said passages to said openings to unplug the same.

ROBERT DOAT.

**References Cited in the file of this patent**

UNITED STATES PATENTS

| Number    | Name          | Date          |
|-----------|---------------|---------------|
| 555,961   | Lungwitz      | Mar. 10, 1896 |
| 591,524   | Burgess       | Oct. 12, 1897 |
| 712,615   | Stapf         | Nov. 4, 1902  |
| 972,126   | Munson        | Oct. 4, 1910  |
| 1,419,764 | Pazos y Sacio | June 13, 1922 |
| 1,502,793 | Maguet        | July 29, 1924 |
| 1,568,364 | Clinginsmith  | Jan. 5, 1926  |
| 1,934,081 | Moll et al.   | Nov. 7, 1933  |
| 2,480,473 | Johnson       | Aug. 30, 1942 |
| 2,504,185 | Debenham      | Apr. 18, 1950 |
| 2,564,009 | Hyche         | Aug. 14, 1951 |
| 2,599,185 | Lipp et al.   | June 3, 1952  |